

Aug. 25, 1936.

A. M. LANE

2,052,032

METAL WEATHER STRIP

Filed Dec. 9, 1935

Fig. 1.



Fig. 2.



Fig. 3.



INVENTOR:

Alfred M. Lane,  
by Ian Alan Spravely.

HIS ATTORNEYS.

## UNITED STATES PATENT OFFICE

2,052,032

## METAL WEATHER STRIP

Alfred M. Lane, St. Louis County, Mo., assignor  
to Monarch Metal Weatherstrip Corporation,  
St. Louis, Mo., a corporation of Missouri

Application December 9, 1935, Serial No. 53,477

5 Claims. (Cl. 20—69)

The ordinary type of metal weatherstrip for a sliding sash comprises two metal strips, one of which has a portion shaped to form a groove and is commonly called the groove strip and the other of which has a portion formed into a rib or bead to fit into said groove and is commonly called the rib strip or bead strip. On account of the exacting requirements for the manufacture and use of such metal weatherstrips, the only materials that could heretofore be successfully used for such metal weatherstrips are zinc and bronze, each of which has many properties that tend to fit them for such purpose. It is important that the metal shall be suitable for shaping rigid grooves therein by rolling or other ordinary manufacture operation, without substantial distortion, and that the metal withstand bending, the finished weatherstrip in some cases having portions doubled back against each other. It is also important that the metal have a negligible amount of creep at the operating stresses and under normal operating temperatures to which weatherstrips are subjected so that the finished weatherstrips shall be resilient, capable of sliding on each other without excessive friction and without galling the surfaces thereof and resistant to atmospheric conditions. In addition to these properties, which are possessed by zinc and certain bronzes to a practicable extent, it is desirable that the metal should be of an ornamental color and that it should resist accumulation of dirt thereon and that it should be more economical. The principal object of the present invention is to produce metal weatherstrips that will embody all of these properties. The invention consists principally in metal weatherstrips made of strips of aluminum alloy having the above mentioned characteristics and having an oxide coating and impregnated with paraffin or other material having lubricating properties. The term "oxide coating" as used herein defines those oxide coatings which are produced on the surface of aluminum or its alloys by the action of some chemical agent with or without the aid of the electric current. It does not include the very thin film of aluminum oxide which is normally formed upon the metal by contact with the air. As at present advised, sulfuric acid is the preferred oxide coating forming agent, but there are many other chemicals and chemical agents which produce, either with or without the external application of electrical energy, an oxide coating upon the surface of aluminum and its alloys. While all such coatings are similar in chemical composition their physical properties reflect to some extent those of the ox-

ide coating forming agent which is used. Chromic acid and oxalic acid are examples of oxide coating forming agents which with the use of externally applied electrical energy produce satisfactory coatings for my purpose. An example of an oxide coating forming agent which may be used without the application of electrical energy is a mixture of sodium carbonate and potassium dichromate.

In the accompanying drawing which illustrates my invention as embodied in a metal weatherstrip of old type,

Fig. 1 is a perspective view of the groove strip,

Fig. 2 is a perspective view of the head strip, and

Fig. 3 is a sectional view of the assembled weatherstrip mounted in a window.

The metal weatherstrip illustrated in the accompanying drawing comprises a groove strip 1 and a bead strip 2. The bead strip has a portion 20 of the metal shaped into a longitudinal bead or rib whose outer portion is of circular or pear-shaped section spaced from the body of the strip by a short neck or connecting portion. The groove strip has a portion formed into a longitudinal groove of proper size and shape to fit freely over the bead of the bead strip. The construction described is typical of existing weatherstrips and may be modified in accordance with common practice.

According to the present invention, the groove strip and the bead strip are made of strips of aluminum or aluminum alloy whose contacting surfaces have been given an oxide coating having a depth of one to two ten thousandths of an inch. 35 This coating is very hard and constitutes a continuous coating over the surface of the aluminum, to which it adheres with great tenacity. This aluminum oxide surface is minutely porous, that is, it is filled with a multiplicity of very minute 40 pores. The oxide coating is indicated by C in the drawing, the thickness thereof being exaggerated for purposes of illustration.

A suitable aluminum alloy for the purpose is one containing small quantities of magnesium (2.5% 45 being a satisfactory content) with or without smaller quantities of chromium (.25% being a satisfactory content).

A suitable process for producing the oxide coating on the aluminum or aluminum alloy is to treat 50 the material anodically with low working voltages (say from 6 to 20 volts) in a bath of sulfuric acid having a concentration of from 15 to 35 percent by weight.

After the material has been given its oxide 55

- coating, it is treated with paraffin, greasy matter such as lanolin or other lubricating substance. I prefer to dip the material into a bath of paraffin at a temperature high enough to liquefy the paraffin. The material is then cooled and the excess paraffin is then wiped off. If the aluminum has been treated in strip form, it is ready for manufacture into metal weather-stripping, if in sheet form, it must first be cut into strips.
- 10 Aluminum weatherstrips made in accordance with my invention and having on their surface an oxide coating impregnated with a lubricant are capable of sliding one on the other without excessive friction and without surface galling.
- 15 They are resistant to atmospheric condition and in fact, the wear due to this sliding action is slower than in the case of zinc and bronze strips. Among the advantages of weatherstrips made of paraffined and oxidized aluminum alloy are the
- 20 following: They require less force to slide sashes equipped therewith; are more durable than zinc and bronze strips; they are substantially free from corrosion and burnishing; they have a pleasing color; they tend to repel ordinary dirt and are
- 25 more readily cleanable than zinc and bronze.
- While I have had very satisfactory results with impregnating a surface portion of the coated aluminum alloy with a solution of paraffin in naptha having specific gravity of .74 degrees
- 30 Baumé, (ten percent by weight of paraffin in naptha) I do not wish to be restricted to such paraffin. The surface portion of the coated aluminum alloy, with its highly minutely porous structure, has a high capacity for absorbing and
- 35 retaining oily and greasy matter. In fact I have found that it will take up and retain carbon black or finely divided graphite in sufficient quantities to overcome the tendency for strips to gall and

stick together. Graphite and paraffin are of mineral origin and, together with carbon black, have the important property of being inert as to oxygen at atmospheric temperature, whereas many animal and vegetable oils oxidize and become 5 gummy when exposed to the atmosphere for a considerable length of time. Likewise, paraffin, graphite and carbon black are unaffected by or highly resistant to atmospheric gases such as carbonic acid, sulphuric acid and ammonia.

10

The term aluminum in the claims is to be understood as meaning either aluminum alloy or aluminum.

What I claim is:

1. A metal weatherstrip consisting of aluminum 15 whose surface portion has an oxide coating impregnated with a lubricant which is resistant to reaction with atmospheric gases.

2. A metal weatherstrip consisting of aluminum 20 whose surface portion has an anodic oxide coating impregnated with a lubricant which is inert as to oxygen at atmospheric temperature.

3. A metal weatherstrip whose body consists of aluminum having a layer of highly and minutely porous oxide of aluminum thereon, said aluminum 25 oxide being impregnated with oily or greasy material of mineral origin.

4. A metal weatherstrip whose body consists of aluminum having a layer of highly and minutely porous oxide of aluminum thereon, said aluminum 30 oxide being impregnated with paraffin.

5. A metal weatherstrip whose body consists of formed aluminum having a layer of highly and minutely porous oxide of aluminum thereon, said aluminum 35 oxide being impregnated with carbon black.

ALFRED M. LANE.